# EUROPEAN PATENT SPECIFICATION

(11) **EP 2 272 994 B1**
(45) Date of publication and mention of the grant of the patent: **12.11.2014**
(21) Application number: 09726619.1
(22) Date of filing: 27.03.2009
(51) Int. Cl.: C22C 38/14, C22C 38/58, C21D 8/02

(54) **HIGH-TENSILE STRENGTH STEEL AND MANUFACTURING METHOD THEREOF**
STAHL MIT HOHER BRUCHFESTIGKEIT UND HERSTELLUNGSVERFAHREN DAFÜR
ACIER AYANT UNE RÉSISTANCE À LA TRACTION ÉLEVÉE ET SON PROCÉDÉ DE FABRICATION

(30) Priority: 31.03.2008 JP 2008089648
(43) Date of publication of application: 12.01.2011
(73) Proprietor: JFE Steel Corporation, Tokyo 100-0011 (JP)
(72) Inventor: ICHIMIYA, Katsuyuki, Tokyo 100-0011 (JP); YOKOTA, Tomoyuki, Tokyo 100-0011 (JP); NISHIMURA, Kimihiro, Tokyo 100-0011 (JP); SHIKANAI, Nobuo, Tokyo 100-0011 (JP)
(74) Representative: Stebbing, Timothy Charles
(86) International application number: PCT/JP2009/056906
(87) International publication number: WO 2009/123292

(56) References cited:
- EP-A1- 1 354 973
- EP-A1- 1 533 392
- EP-A1- 1 870 484
- WO-A1-2007/023804
- CN-A- 101 151 393
- DE-A1- 3 142 782
- JP-A- 58 077 529
- JP-A- 63 210 235
- JP-A- 2002 212 670
- JP-A- 2002 235 114
- JP-A- 2002 317 242
- JP-A- 2007 231 312
- JP-A- 2007 277 681

## Description

### Technical Field

The present invention relates to a method of manufacturing a high-tensile strength steel that is used in ships, marine structures, line pipes, pressure vessels. Specifically, the present invention relates to a method of manufacturing a high-tensile strength steel that has a yield stress (YS) of 460 MPa or more and is not only excellent in strength and toughness of base material but also excellent in weld zone toughness (crack tip opening displacement (CTOD) properties).

### Background Art

Steels used in ships, marine structures, and so on are usually formed into structures having desired shapes by welding joints. Therefore, from the viewpoint of ensuring safety of structures and so on, it is required not only that the base material itself is excellent in strength and toughness but also that the weld zone (weld metal and heat-affected zone) of a weld joint is excellent in toughness.

As evaluation standards of toughness of steels, conventionally, absorbed energy in a Charpy impact test has been mainly used. However, recently, in order to increase the reliability, a crack tip opening displacement test (hereinafter abbreviated to "CTOD test") is often used. In this test, a test piece having a fatigue precrack in a toughness-evaluating portion is subjected to three-point bending, and the value of opening displacement (value of plastic deformation) of the bottom of crack immediately before breaking is measured to evaluate occurrence resistance of brittle fracture.

Generally, steels having large thicknesses, as in those used in the above-mentioned purposes, are usually subjected to multi-pass welding. In such welding, since the heat-affected zone experiences a complicated thermal history, there are problems that local embrittlement tends to occur and that, in particular, the bond zone (boundary between a weld metal and a base material) and the inter-critically reheated zone (region that is coarse-grained in the first cycle of welding and is heated into a two-phase region of a and y in the second cycle) are largely decreased in toughness. This is because that since the bond zone is exposed to a high temperature just below the melting point, austenite grains are coarsened and are, by subsequent cooling, transformed into a brittle upper bainitic structure. In addition, in the bond zone, embrittlement structures such as a Widmannstatten structure and island martensite (Martensite-Austenite constituent) are formed, and thereby the toughness is further deteriorated.

As a countermeasure against the problems mentioned above, for example, a technique of finely dispersing TiN in a steel in order to prevent the coarsening of austenite grains or to use as nuclei of ferrite transformation has been put into practical use. Furthermore, Japanese Examined Patent Application Publication No. 03-053367 and Japanese Unexamined Patent Application Publication No. 60-184663 disclose techniques of dispersing fine particles in a steel by combined addition of a rare-earth metal (REM) and Ti for preventing the growth of austenite grains and improving the toughness of the weld zone. In addition to the above, proposed are a technique of dispersing an oxide of Ti, a technique of combining ferrite nucleus-forming ability of BN with oxide dispersion, and also a technique of increasing toughness by controlling the shape of sulfide by adding Ca or REM.

The inter-critically reheated zone, that is, a region that is exposed to a high temperature just below the melting point in the first welding and is reheated to a two-phase region of ferrite and austenite in the subsequent welding is most embrittled. This is because that carbon is enriched in the austenite region by reheating to a two-phase region, and this allows the formation of a brittle bainitic structure containing island martensite during cooling, resulting in a decrease in toughness. Accordingly, as a countermeasure against the above, a technique of preventing the formation of island martensite by reducing the amounts of C and Si and also ensuring the base material strength by adding Cu is disclosed (for example, Japanese Unexamined Patent Application Publication No. 05-186823).

Furthermore, Japanese Unexamined Patent Application Publication No. 2007-231312 discloses, as a method for preventing the formation of an embrittlement structure due to reheating in welding, a technique of increasing the toughness of the welded heat-affected zone (CTOD properties) by adding Ni, while adjusting the amount of Ca added for controlling the shape of sulfide within an appropriate range.

However, though the problem of a reduction in toughness of the heat-affected zone is improved to a certain extent by the above-described conventional techniques, some problems to be solved are left. For example, in the technique using TiN, the effect is lost in the bond zone that is heated to a temperature range at which TiN is dissolved, and also a significant decrease in toughness may occur by embrittlement of the base structure due to a Ti solid solution and a N solid solution. The technique of using an oxide of Ti has a problem that the fine dispersion of the oxide cannot be sufficiently uniform. Furthermore, recently, along with an increase in size of ships and marine structures, steels used therein are required to have higher strengths and larger thicknesses. In order to correspond to these requirements, on the contrary to the technique of Japanese Unexamined Patent Application Publication No. 05-186823, it is effective to add large amounts of alloy elements. However, the addition of large amounts of alloy elements causes the formation of an embrittlement structure and thus decrease in toughness of the welded heat-affected zone. Furthermore, in the technique disclosed in Japanese Unexamined Patent Application Publication No. 2007-231312, the addition of Ni, which is effective for increasing the toughness of a matrix (effect of a Ni solid solution), is indispensable as a measure for increasing the strength and the thickness, which causes a problem of an increase in cost.

Other prior art proposals for a high-tensile strength steel include JP 2002 235 114 CN 101151393 A, EP 1 870 484 A1 and EP 1 533 392 A1 by the present applicant, EP 1 354 973 A1 by Nippon Steel Corp., and WO 2007/023804 A1 by Sumitomo Metal Industries et al.

Accordingly, it is an object of the present invention to solve the problems of the conventional techniques and thereby to propose a high-tensile strength steel that is not only excellent in strength and toughness of the base material but also excellent in toughness of the welded heat-affected zone, even in thick high-strength steel plate that are necessarily increased in the amounts of alloy elements, and to propose a method of properly manufacturing the steel.

### Disclosure of Invention

The present invention provides a method of manufacturing a high-tensile strength steel comprising:
heating a steel slab having a component composition including C: 0.03 to 0.10 mass%, Si: 0.30 mass% or less, Mn: 1.60 to 2.30 mass%, P: 0.015 mass% or less, S: 0.005 mass% or less, Al: 0.005 to 0.06 mass%, Nb: 0.004 to 0.05 mass%, Ti: 0.005 to 0.02 mass%, N: 0.001 to 0.005 mass%, Ca: 0.0005 to 0.003 mass%, and optionally further comprising one or more selected from the group consisting of B: 0.0003 to 0.0025 mass%, V: 0.2 mass% or less, Cu: 1 mass% or less, Ni: 2 mass% or less, Cr: 0.7 mass% or less, and Mo: 0.7 mass% or less, and the balance of Fe and inevitable impurities so that Ca, S, and O satisfy the following expression (1):

   0 < (Ca-(0.18+130xCa)xO)/1.25/S < 1 (1)

   wherein, Ca, S, and O represent the respective contents (mass%) of the elements, to 1050 to 1200 °C;
   hot-rolling the steel in such a manner that the cumulative rolling reduction in the temperature range of 950°C or higher is 30% or more and the cumulative rolling reduction in the temperature range of lower than 950°C is 30 to 70%; and then
   cooling the steel from the hot-rolling finishing temperature to a cooling termination temperature of 600 to 450°C at a cooling rate of 5 to 45°C/sec and then cooling the steel from the former cooling termination temperature to a cooling termination temperature of 450°C or lower at a cooling rate of 1°C/sec or more and less than 5°C/sec.

Furthermore, the manufacturing method of the present invention can subject the steel after the latter cooling to tempering at 450 to 650°C.

The first cooling is preferably performed at a cooling rate of 5 to 20°C/sec.

According to the present invention, a high-strength steel where the base material has a high strength with a yield stress of 460 MPa or more and is excellent in toughness and also the heat-affected zone after welding is excellent in toughness (CTOD properties) can be manufactured inexpensively.

Therefore, the invention highly contributes to an increase in size of ships, marine structures, and so on.

### Brief Description of Drawings

[Fig. 1] Fig. 1 is a graph showing an effect of the first cooling rate (cooling rate from the finishing rolling temperature to a cooling termination temperature of 600 to 450°C) after hot-rolling on base material properties.

### Best Modes for Carrying Out the Invention

The present inventors have intensively investigated methods that can increase the strength and toughness of the base material of a thick high-tensile strength steel and also improve the toughness of the welded heat-affected zone. As a result, it has been found that since a decrease in toughness of a welded heat-affected zone is caused by formation of an embrittlement structure, in order to increase the toughness of the welded heat-affected zone, prevention of coarsening of austenite grains in a region that is heated to a high temperature in welding and also uniform and fine dispersion of transformation nuclei for accelerating ferrite transformation in cooling after the welding are effective.

Accordingly, the present inventors have further investigated methods for preventing the formation of embrittlement structures and, as a result, have found the facts that adjustment of the amount of Ca added for controlling the shape of sulfide to an appropriate range is effective and that addition of Mn is effective for increasing the toughness (CTOD properties) of a welded heat-affected zone.

Furthermore, effects of rolling conditions on the strength and toughness of base materials have been investigated, and, as a result, it has been found that a steel plate of which main structure is an acicular ferrite structure can be obtained by conducting cooling after rolling by two-stage cooling consisting of first cooling at a high cooling rate and then cooling at a low cooling rate and appropriately controlling both the cooling rates, and thereby a high-tensile strength steel excellent in strength and toughness of the base material can be manufactured. Furthermore, it has been found that, in order to further increase the strength and toughness of the base material, it is important to effectively use Nb, which is highly effective for forming a non-recrystallization zone in a low temperature range of austenite. Thus, the present invention has been finally accomplished by appropriately combining these techniques.

The basic technological concept of the present invention will be described.

A first aspect of the present invention is that, in order to increase the toughness of the welded heat-affected zone, crystallization of a compound (CaS) of Ca added for controlling the shape of sulfide is effectively utilized. Since the CaS is crystallized at a lower temperature compared to oxide, its uniform fine dispersion is possible. In addition, since a S solid solution is ensured even after crystallization of CaS by controlling the CaS addition amount and the dissolved oxygen amount in a molten steel when it is added to an appropriate ranges, MnS is precipitated on the surface of CaS to form complex sulfide. It is known that MnS has potential for ferrite nucleus, and a Mn depleted zone is formed in the periphery of precipitated MnS. Therefore, ferrite transformation is further accelerated. This effect of the Mn depleted zone can be further effectively exhibited by increasing the amount of Mn added to the steel. In addition, ferrite transformation nuclei such as TiN, BN, or AlN are precipitated on the precipitated MnS, which accelerates further ferrite transformation.

In addition, an increase in the Mn addition amount can effectively increase the base material strength in such a manner that island martensite, which is an embrittlement structure, is not formed as far as possible in the welded heat-affected zone. This is because that the island martensite formed during the cooling after welding tends to be decomposed to cementite by increasing the Mn addition amount thereby to reduce the island martensite in the heat-affected zone structure. As a result of these effects, the toughness of the welded heat-affected zone can be ensured without requiring addition of Ni.

According to the technique described above, ferrite transformation nuclei that are not dissolved even at high temperature can be finely dispersed thereby to reduce the welded heat-affected zone structure in size, and also high toughness can be obtained by preventing the formation of island martensite (M-A constituent) as far as possible. In addition, since the first welded heat-affected zone structure is reduced in size, even in the region reheated into two-phase region by a heat cycle in multilayer welding, the toughness of the untransformed region is increased. Furthermore, since the austenite grains that are retransformed are also reduced in size, the degree of a decrease in toughness can be controlled to be small.

A second aspect of the present invention is that the cooling after rolling of a steel is performed by two-stage cooling of former cooling and latter cooling, wherein the cooling rate of the first cooling is higher than that of the second cooling. This point will be described on the basis of experimental results.

A steel slab including C: 0.08 mass%, Si: 0.2 mass%, and Mn: 1.8 mass% as basic components was heated to 1150°C and then hot-rolled in such a manner that the cumulative rolling reduction in the temperature range of 950°C or higher was 40%, the cumulative rolling reduction in the temperature range of lower than 950°C was 50%, and the finishing rolling temperature was 850°C, and then first cooling for cooling the steel from the rolling completion temperature to 500°C at a cooling rate of 5 to 45°C/sec, more preferably, 5 to 20°C/sec, and then cooling for cooling the steel to 350°C at a cooling rate of 3°C/sec were performed, followed by air cooling to give a thick steel sheet having a thickness of 10 to 50 mm. The thick steel plate was examined for tensile strength properties and toughness properties at -40°C (Charpy impact absorbed energy).

Regarding the results of the measurement, Fig. 1 shows an effect of former cooling rate on the strength and toughness of the base material. It is confirmed that a steel excellent in strength-toughness balance such that the strength is high so as to have a yield stress of 460 MPa or more and the vE-40°C is 200 J or more can be obtained by controlling the cooling rate of the first cooling from the finishing rolling temperature to 500°C to the range of 5 to 45°C/sec.

Furthermore, it was confirmed that the main microstructure of the steel plate thus cooled at the above-mentioned cooling rate is acicular ferrite. In general, when a high strength steel is tried to be obtained, a relatively coarse upper bainitic microstructure that contains, for example, island martensite between laths is formed, resulting in a large decrease in toughness. Accordingly, in order to achieve both high strength and high toughness, it is necessary to form a finer acicular ferrite microstructure by, for example, adjusting the rolling conditions. However, the present inventors have found the fact that a steel sheet excellent in strength-toughness balance can be obtained by performing the cooling after rolling by two steps of former cooling and latter cooling, wherein the cooling rate of the second cooling is lower than that of the first cooling and both the cooling rates are appropriately controlled, thereby to form a structure of mainly acicular ferrite. This is because that the microstructure after transformation can become a dense acicular ferrite instead of a coarse bainitic microstructure by performing the first cooling at a higher cooling rate than that of the second cooling to increase the transformation nucleation density. Furthermore, it has been found that the cooling rate of the second cooling is required to be controlled in an appropriate range because that when the cooling rate is too higher than that of the first cooling, island martensite is formed to decrease the toughness of the base material and, in contrast, that when the cooling rate of the second cooling is too low, the strength of the base material is decreased.

The present invention has been thus accomplished based on the above-described findings.

Next, the chemical composition that should be possessed by the high-tensile strength steel according to the present invention will be described.

### C: 0.03 to 0.10 mass%

C is an element that most largely affects the strength of a steel and is necessary to be contained in an amount of 0.03 mass% or more for ensuring strength (YS ≥ 460 MPa) required in structural steels. However, conversely, when the amount is too large, a decrease in toughness of the base material and cold cracking during welding are caused. Therefore, the upper limit is determined to be 0.10 mass%.

### Si: 0.30 mass% or less

Si is a component that is added as a deoxidizing material and also for highly strengthening a steel. In order to obtain such effects, it is preferable that the addition amount be 0.01 mass% or more. However, when the amount is higher than 0.30 mass%, the toughness of the base material and the weld zone is reduced. Therefore, the amount has to be 0.30 mass% or less and is preferably in the range of 0.01 to 0.20 mass%.

### Mn: 1.60 to 2.30 mass%

Mn is an element effective for ensuring the strength of the base material, but, in the present invention, Mn is an important element that is added for accelerating the reduction of a welded heat-affected zone structure in size and also preventing the formation of an embrittlement structure as far as possible thereby to increase the toughness of the welded heat-affected zone (CTOD properties). In order to achieve these effects, an addition amount of 1.60 mass% or more is necessary. Conversely, since an amount larger than 2.30 mass% significantly decreases the toughness of the base material and the weld zone, the amount is 2.30 mass% or less and is preferably in the range of 1.65 to 2.15 mass%.

### P: 0.015 mass% or less

P is an impurity that is inevitably contained. When the amount is larger than 0.015 mass%, the toughness of the base material and the weld zone is decreased, and therefore the amount is limited to 0.015 mass% or less and preferably 0.010 mass% or less.

### S: 0.005 mass% or less

S is an impurity that is inevitably contained. When the amount is larger than 0.005 mass%, the toughness of the base material and the weld zone is decreased, and therefore the amount is limited to 0.005 mass% or less and preferably 0.0035 mass% or less.

### Al: 0.005 to 0.06 mass%

Al is an element to be added for deoxidizing the molten steel and is required to be contained in an amount of 0.005 mass% or more. On the other hand, an amount larger than 0.06 mass% decreases the toughness of the base material and also causes interfusion with a weld metal by dilution due to welding, which decreases the toughness. Therefore, the amount is necessarily limited to 0.06 mass% or less and preferably 0.010 to 0.055 mass%.

### Nb: 0.004 to 0.05 mass%

Nb enlarges a non-recrystallization zone in a low temperature range of austenite. Therefore, the base material structure can be reduced in size and increased in toughness by conducting rolling in such a temperature range. In addition, precipitation strengthening can be achieved by conducting tempering after the rolling and cooling. Therefore, Nb is an important element from the viewpoint of strengthening the steel. In order to obtain the above-described effects, Nb is necessarily contained in an amount of 0.004 mass% or more. However, when Nb is added in an excessive amount of higher than 0.05 mass%, the toughness of the weld zone is decreased. Therefore, the upper limit is determined to be 0.05 mass%.

### Ti: 0.005 to 0.02 mass%

Ti is precipitated as TiN when molten steel is solidified thereby to prevent the austenite in the weld zone from being coarsened and also acts as ferrite transformation nuclei thereby to contribute to an increase in toughness of the weld zone. In order to obtain the effects, Ti is necessarily contained in an amount of 0.005 mass% or more. When the amount is less than 0.005 mass%, the effect is small, but an amount larger than 0.02 mass% causes coarsening of TiN grains, and, thereby, the effect increasing the toughness of the base material and the weld zone cannot be obtained. Therefore, the Ti addition amount is determined to be in the range of 0.005 to 0.02 mass%.

### N: 0.001 to 0.005 mass%

N is an element necessary for forming TiN that prevents the weld zone structure from being coarsened and is contained in an amount of 0.001 mass% or more. On the other hand, when the amount is larger than 0.005 mass%, the N solid solution significantly decreases the toughness of the base material and the weld zone. Therefore, the upper limit is determined to be 0.005 mass%. Incidentally, in order to form TiN in an amount sufficient for pinning to prevent the structure from being coarsened, the N amount is preferably in the range of 0.003 to 0.005 mass%.

### Ca: 0.0005 to 0.003 mass%

Ca is an element that increases the toughness by fixing S. In order to realize this effect, it is necessary to be contained in an amount of at least 0.0005 mass%. However, in an amount larger than 0.003 mass%, the effect is saturated. Therefore, Ca is contained in the range of 0.0005 to 0.003 mass%. $0 < \left(Ca-\left(0.18+130\times Ca\right)\times O\right) / 1.25 / S < 1$

In order to finely disperse CaS serving as a ferrite transformation nucleus that is not dissolved even at high temperature, Ca, S, and O are necessarily contained so as to satisfy the following expression (1): $0 < \left(Ca-\left(0.18+130\times Ca\right)\times O\right) / 1.25 / S < 1$
wherein, Ca, S, and O represent the respective contents (mass%) of the elements. In the expression, (Ca-(0.18+130×Ca)×O)/1.25/S) is a value showing the ratio of atomic concentrations of Ca and S for effectively controlling the shape of sulfide and suggests the shape of the sulfide (Mochida, et al., "Tetsu to Hagane (Iron and Steel)", The Iron and Steel Institute of Japan, vol. 66 (1980), No. 3, pp. 354-362).

That is, when the value of ((Ca- (0.18+130×Ca)×O)/1.25/S) is 0 or less, CaS is not crystallized. Therefore, since S is precipitated in a MnS form alone, fine dispersion of ferrite transformation nuclei in the welded heat-affected zone, which is the focus of the present invention, cannot be achieved. Furthermore, MnS precipitated alone is elongated in rolling process, resulting in a decrease in toughness of the base material.

On the other hand, when the value of ((Ca-(0.18+130×Ca)×O)/1.25/S) is 1 or more, S is completely fixed with Ca, and MnS that acts as a ferrite transformation nucleus is not precipitated on CaS. Therefore, complex sulfide cannot sufficiently act as a ferrite transformation nucleus.

Compared with the above, when Ca, S, and O satisfy the expression (1), MnS is precipitated on CaS to form complex sulfide and can effectively function as a ferrite transformation nucleus. Incidentally, the value of ((Ca-(0.18+130xCa)xO)/1.25/S) is preferably in the range of 0.2 to 0.8.

The high-tensile strength steel of the present invention can contain one or more selected from the group consisting of B, V, Cu, Ni, Cr, and Mo for further increasing strength and toughness, in addition to the above-described essential components.

### B: 0.0003 to 0.0025 mass%

B segregates in an austenite grain boundary and thereby to prevent ferrite transformation that occurs from the grain boundary, which increases the fraction of a bainitic structure thereby to achieve an effect of strengthening the steel. Such an effect can be achieved when the addition amount is 0.0003 mass% or more. However, when the amount is larger than 0.0025 mass%, conversely, the toughness is decreased. The amount of B is more preferably in the range of 0.0005 to 0.002 mass%.

### V: 0.2 mass% or less

V is an element effective for increasing the strength and toughness of the base material and is precipitated as VN, which also acts as a ferrite transformation nucleus. In order to obtain the effects, the amount to be added is preferably 0.01 mass% or more. However, when the addition amount is larger than 0.2 mass%, contrarily, a decrease in toughness is caused. Therefore, the amount to be added is preferably 0.2 mass% or less, and more preferably 0.15 mass% or less.

### Cu: 1 mass% or less

Cu is an element having an effect of increasing the strength of a steel. In order to obtain the effect, it is preferably to be contained in an amount of 0.05 mass% or more. However, when the amount is larger than 1 mass%, hot brittleness causes surface defects of the steel plate. Therefore, the addition amount is preferably in the range of 1 mass% or less and more preferably 0.8 mass% or less.

### Ni: 2 mass% or less

Ni is an element effective for increasing the strength of a steel and the CTOD properties of the welded heat-affected zone. In order to obtain the effects, the addition amount is preferably 0.05 mass% or more. However, since Ni is an expensive element, it is preferably to determine the upper limit to be 2.0 mass%. When the Mn addition amount is 1.6 % or more as in this application, the amount of Ni is further preferably less than 0.3% from the viewpoint of a reduction in cost.

### Cr: 0.7 mass% or less

Cr is an element effective for strengthening the base material. In order to obtain the effect, the addition amount is preferably 0.05 mass% or more. However, since a large amount of Cr, adversely affects the toughness, the upper limit is preferably determined to be 0.7 mass%, more preferably, 0.5 mass% or less.

### Mo: 0.7 mass% or less

Mo is an element effective for strengthening the base material as in Cr. In order to obtain the effect, the addition amount is preferably 0.05 mass% cr more. However, since a large amount of Mo, adversely affects the toughness, the upper limit is preferably determined to be 0.7 mass%, more preferably, 0.5 mass% or less.

Next, the high-tensile strength steel structure of the present invention will be described.

Microstructure of the high-tensile strength steel of the present invention is mainly composed of an acicular ferrite, and its area ratio is preferably 60% or more and more preferably 70% or more. If the area ratio of the acicular ferrite is less than 60% and a coarse upper bainite is increased, the toughness is decreased. Incidentally, the upper limit of the area ratio is not particularly limited. The acicular ferrite microstructure of the high-tensile steel of the present invention is bainitic ferrite with a high dislocation density having morphology of fine needle-like or lath-like shape and is different from a polygonal ferrite or coarse upper bainite.

Next, the method of manufacturing the high-tensile strength steel of the present invention will be described.

It is preferable that the high-tensile strength steel of the present invention be manufactured as a high-tensile strength steel having a large thickness by ingoting a molten steel having the above-described component composition of the present invention by a common method using a converter furnace, an electric furnace, a vacuum melting furnace, or the like, making a steel material such as a slab by a common step such as continuous-casting or ingot-casting-blooming, and then hot-rolling the steel material. On this occasion, it is necessary to adjust the heating temperature of the steel material to the range of 1050 to 1200°C in advance the hot-rolling. A heating temperature of not lower than 1050°C is necessary for certainly pressure-bonding cast defects, which are present in the as-cast steel material, by the hot-rolling. However, since heating to a temperature higher than 1200°C coarsens TiN that has been precipitated during solidification and decreases the toughness of the base material and the weld zone, the heating temperature is necessarily regulated to 1200°C or less.

Then, the steel material heated to the above-mentioned temperature is subjected to hot-rolling in such a manner that the cumulative rolling reduction in the temperature range of 950°C or higher is 30% or more and the cumulative rolling reduction in the temperature range of lower than 950°C is 30 to 70% to obtain a high-tensile strength steel having a set thickness. The hot-rolling is performed at a cumulative rolling reduction of 30% in the temperature range of 950°C or higher because that the austenite grains are recrystallized to make the microstructure fine by regulating the cumulative rolling reduction in this temperature range to 30% or more, but the abnormally coarsened grains produced in the heating are left when the cumulative rolling reduction is lower than 30% to adversely affect the toughness of the base material.

In addition, the hot-rolling is performed at a cumulative rolling reduction of 30 to 70% in the temperature range of lower than 950°C because that since the austenite grains rolled in this temperature range are not sufficiently recrystallized thereby to hold the elongated shape after the rolling, a large amount of defects such as deformation bands are introduced, and thereby the internal strain becomes high. In addition, the cumulative internal energy works as a driving force for the subsequent ferrite transformation to accelerate the ferrite transformation. However, when the cumulative rolling reduction is lower than 30%, the cumulative internal energy is not sufficient. Therefore, the ferrite transformation hardly occurs thereby to decrease the toughness of the base material. On the other hand, a cumulative rolling reduction of higher than 70% accelerates the formation of polygonal ferrite and prevents the formation of acicular ferrite, and, therefore, high strength and high toughness cannot be simultaneously achieved.

The subsequent cooling after the completion of the hot-rolling is performed by a first cooling and a second cooling, and the cooling rate of the first cooling is relatively higher than that of the second cooling. That is, it is necessary that the first cooling is performed from the finishing rolling temperature to a cooling termination temperature of 600 to 450°C, preferably, from the finishing rolling temperature to a cooling termination temperature of 580 to 480°C at a cooling rate of 5 to 45°C/sec, preferably 5 to 20°C/sec, and further preferably 6 to 16°C/sec, and then the second cooling is performed from the first cooling termination temperature to the second cooling termination temperature of 450°C or less, preferably, from the first cooling termination temperature to the cooling termination temperature of 400 to 250°C at a cooling rate of 1°C/sec or more and less than 5°C/sec, more preferably, 2 to 4.5°C/sec.

When the cooling termination temperature of the first cooling is higher than the above-mentioned temperature range, the strength is hardly increased. Conversely, when the temperature is lower than the above-mentioned temperature range, the toughness is deteriorated. In addition, when the first cooling rate is lower than the lower limit of the above-mentioned range, the dominant microstructure is polygonal ferrite, and therefore an increase in the strength is not obtained. Conversely, when the rate is higher than the upper limit of the above-mentioned range, the toughness is decreased. Furthermore, when the cooling termination temperature of the second cooling is higher than the upper limit of the above-mentioned temperature range, the increase of the strength is insufficient. In addition, the second cooling rate is lower than the lower limit of the above-mentioned range, the base material suffers from a shortage of strength. Conversely, when the rate is higher than the upper limit of the above-mentioned range, the toughness of the base material is decreased. In addition, when the latter cooling rate is too higher than that of the first cooling rate, island martensite is formed thereby to decrease the toughness of the base material.

Incidentally, in the present invention, in order to reduce the residual internal stress, the steel material after the cooling may be subjected to tempering in the temperature range of 450 to 650°C. When the temperature of the tempering is lower than 450°C, the effect removing the residual stress is small. On the other hand, when the temperature is higher than 650°C, various types of carbonitrides are precipitated thereby to cause precipitation strengthening and decrease the toughness, which is undesirable.

As described above, in the method of manufacturing a high-tensile strength steel of the present invention, it is important to appropriately control the cumulative rolling reduction according to the rolling temperature in the hot-rolling and to appropriately control the two-stage cooling conditions after the completion of the rolling. In particular, by setting the cooling rate of the first cooling to be larger than that of the second cooling, the main structure of the base material becomes acicular ferrite, and thereby a steel material excellent in strength-toughness balance can be obtained.

Furthermore, in the present invention, a high strength steel in which the base material has a high strength of a yield stress of 550 MPa or more and is excellent in toughness and also the heat-affected zone after welding is excellent in toughness (CTOD properties) can be inexpensively manufactured by controlling the amount of N in the chemical components to be higher than 0.0030%, the cooling rate in the former cooling to higher than 20°C/sec and not higher than 45°C/sec, the cooling termination temperature of the former cooling to 450°C or higher and lower than 500°C.

### Example

Thick steel sheets having thicknesses of 25 to 80 mm were manufactured using steel slabs Nos. 1 to 31 having component compositions shown in Tables 1-1 and 1-2 as materials by performing hot-rolling, former cooling, and latter cooling under conditions shown in Tables 2-1 and 2-2. Incidentally, the temperatures shown in Tables 2-1 and 2-2 are each that of one-fourth thickness portion calculated from the steel plate surface temperature measured with a radiation thermometer. Samples prepared from the thus obtained thick steel plates were subjected to a tensile test and a Charpy impact test. In the tensile test, JIS #4 tensile test pieces were sampled from one-fourth thickness portions of the thick steel plates in such a manner that the longitudinal axis direction of each test piece was parallel to the rolling direction, and the yield stress (YS) and tensile strength (TS) of the test pieces were measured. In the Charpy impact test, JIS #4 impact test pieces were sampled from one-fourth thickness portions of the thick steel plates parallel to transverse direction, and the absorbed energy at -40°C (vE-40°C) was measured. A test piece satisfying all of YS ≥ 460 MPa, TS ≥ 570 MPa, and vE-40°C ≥ 200 J was determined to have satisfactory base material properties.

Furthermore, test plates prepared from the thick steel plates that satisfy all the above-mentioned criteria of YS, TS, and vE-40°C as the base material properties were each provided with a single bevel groove (bevel angle: 30°). The test plate was subjected to CO₂ arc welding at a heat input amount of 25 kJ/cm to produce a weld joint. A CTOD test piece provided with a notch in the straight bond zone of the single bevel groove was prepared from each weld joint and subjected to a CTOD test at -10°C. Incidentally, the preparation of the CTOD test pieces and the test conditions were in accordance with British standard BS 7448. In addition, JIS #4 impact test pieces having notches in the bond zones were prepared and were each subjected to the Charpy impact test at -40°C and measured for the absorbed energy (vE-40°C).

The test results are also shown in Tables 2-1 and 2-2. These results confirm that in the steel plates of the present invention, the base material has a yield stress (YS) of 460 MPa or more and a Charpy absorbed energy (vE-40°C) of 200 J or more and is thus excellent in both the strength and the toughness, and also the welded heat-affected zone is excellent in toughness such that the bond zone of a CO₂ arc welding joint has a vE-40°C of 200 J or more and a CTOD value of 0.10 mm or more. On the other hand, in Comparative Examples that are out of the scope of the present invention, the resulting steel plates are unsatisfactory in any one or more of the above-mentioned characteristics.

Furthermore, the steel plates of Nos. 11 to 17, which are steel plates according to the present invention and contain N in amounts of larger than 0.0030 mass%, are excellent such that all the CTOD values of weld zones are 0.45 mm or more due to the pinning effect of TiN.

Furthermore, in both the steel plates of Nos. 15 and 16, which are steel plates of the present invention and contain N in amounts of larger than 0.0030 mass% and of which manufacturing conditions are that the cooling rate of the first cooling after hot-rolling is higher than 20°C/sec and not higher than 45°C/sec and the first cooling termination temperature is 450°C or higher and lower than 500°C, the base materials have high strength such that the yield stresses are 550 MPa or more.

### Industrial Applicability

The high-tensile strength steels of the present invention can be properly used not only in ships, marine structures, line pipes, and pressure vessels but also in steel structures that are assembled by welding in the fields of constructions, civil works, and so on.

**Table 1-1**

| No. | Chemical Component (mass%) | | | | | | | | | | | | | | | | | | | Notes |
|---|---|---|---|---|---|---|---|---|---|---|---|---|---|---|---|---|---|---|---|---|
| | C | Si | Mn | P | S | Al | Nb | Ti | N | Ca | O | B | V | Cu | Ni | Cr | Mo | Ceq *1 | ACR *2 | |
| 1 | 0.056 | 0.10 | 2.05 | 0.005 | 0.0018 | 0.026 | 0.030 | 0.019 | 0.0015 | 0.0030 | 0.0035 | - | - | 0.22 | 0.23 | - | - | 0.428 | 0.447 | Example |
| 2 | 0.055 | 0.08 | 2.15 | 0.009 | 0.0015 | 0.044 | 0.029 | 0.017 | 0.0038 | 0.0024 | 0.0017 | - | - | - | - | 0.11 | - | 0.435 | 0.834 | Example |
| 3 | 0.076 | 0.13 | 2.02 | 0.010 | 0.0021 | 0.027 | 0.022 | 0.014 | 0.0028 | 0.0014 | 0.0024 | - | - | - | - | - | 0.20 | 0.453 | 0.202 | Example |
| 4 | 0.077 | 0.08 | 1.99 | 0.009 | 0.0034 | 0.050 | 10.025 | 0.011 | 0.0047 | 0.0023 | 0.0028 | - | - | 0.34 | 0.19 | - | - | 0.444 | 0.226 | Example |
| 5 | 0.063 | 0.18 | 2.12 | 0.005 | 0.0016 | 0.047 | 0.021 | 0.014 | 0.0019 | 0.0019 | 0.0016 | - | - | - | - | 0.21 | - | 0.458 | 0.608 | Example |
| 6 | 0.052 | 0.06 | 2.14 | 0.004 | 0.0026 | 0.016 | 0.034 | 0.018 | 0.0019 | 0.0011 | 0.0012 | 0.0019 | - | - | - | - | - | 0.409 | 0.219 | Example |
| 7 | 0.085 | 0.16 | 2.14 | 0.008 | 0.0019 | 0.030 | 0.033 | 0.017 | 0.0024 | 0.0013 | 0.0022 | - | 0.016 | - | - | - | 0.12 | 0.469 | 0.224 | Example |
| 8 | 0.036 | 0.19 | 1.78 | 0.005 | 0.0026 | 0.017 | 0.019 | 0.015 | 0.0031 | 0.0011 | 0.0012 | - | 0.022 | 0.022 | - | 0.32 | 0.28 | 0.457 | 0.219 | Example |
| 9 | 0.053 | 0.20 | 1.66 | 0.008 | 0.0028 | 0.029 | 0.037 | 0.015 | 0.0033 | 0.0030 | 0.0032 | - | - | - | - | 0.29 | 0.17 | 0.422 | 0.336 | Example |
| 10 | 0.066 | 0.19 | 2.11 | 0.006 | 0.0011 | 0.024 | 0.039 | 0.016 | 0.0022 | 0.0008 | 0.0012 | - | - | - | - | - | - | 0.418 | 0.334 | Example |
| 11 | 0.048 | 0.05 | 1.88 | 0.007 | 0.0026 | 0.033 | 0.008 | 0.012 | 0.0037 | 0.0022 | 0.0018 | - | - | 0.15 | 0.18 | - | - | 0.383 | 0.419 | Example |
| 12 | 0.062 | 0.03 | 1.75 | 0.009 | 0.0035 | 0.028 | 0.026 | 0.014 | 0.0048 | 0.0011 | 0.0021 | - | - | - | - | 0.20 | 0.10 | 0.414 | 0.096 | Example |
| 13 | 0.071 | 0.16 | 2.12 | 0.005 | 0.0015 | 0.043 | 0.016 | 0.008 | 0.0043 | 0.0008 | 0.0028 | - | - | - | - | - | - | 0.424 | 0.003 | Example |
| 14 | 0.055 | 0.12 | 2.06 | 0.012 | 0.0019 | 0.035 | 10.012 | 0.016 | 0.0045 | 0.0016 | 0.0024 | 0.0011 | - | - | - | - | - | 0.398 | 0.282 | Example |
| 15 | 0.050 | 0.08 | 1.98 | 0.011 | 0.0031 | 0.038 | 0.015 | 0.010 | 0.0034 | 0.0022 | 0.0015 | - | - | 0.33 | 0.75 | - | - | 0.452 | 0.387 | Example |

| | | | | | | | | | | | | | | | | | | | | |
|---|---|---|---|---|---|---|---|---|---|---|---|---|---|---|---|---|---|---|---|---|
| *1: Ceq=C+Mn/6+(Cr+Mo+V)/5+(Cu+Ni)/15 *2: ACR=(Ca-(0.18+130×Ca)×0)/1.25/S In expressions *1 and *2, the element symbols represent the respective contents (mass%) of the elements. | | | | | | | | | | | | | | | | | | | | |

**Table 1-2**

| No. | Chemical Component (mass%) | | | | | | | | | | | | | | | | | | | Notes |
|---|---|---|---|---|---|---|---|---|---|---|---|---|---|---|---|---|---|---|---|---|
| | C | Si | Mn | P | S | Al | Nb | Ti | N | Ca | O | B | V | Cu | Ni | Cr | Mo | Ceq*1 | ACR *2 | |
| 16 | 0.015 | 0.18 | 1.72 | 0.006 | 0.0034 | 0.035 | 0.038 | 0.009 | 0.0027 | 0.0015 | 0.0010 | - | - | - | - | - | 0.19 | 0.340 | 0.265 | Comparative Example |
| 17 | 0.130 | 0.13 | 2.07 | 0.007 | 0.0016 | 0.053 | 0.029 | 0.018 | 0.0043 | 0.0022 | 0.0015 | - | - | - | - | - | - | 0.475 | 0.751 | Comparative Example |
| 18 | 0.080 | 0.42 | 2.06 | 0.010 | 0.0029 | 0.048 | 0.043 | 0.014 | 0.0024 | 0.0027 | 0.0012 | - | - | - | - | - | - | 0.423 | 0.569 | Comparative Example |
| 19 | 0.064 | 0.09 | 1.36 | 0.006 | 0.0025 | 0.028 | 0.016 | 0.012 | 0.0049 | 0.0030 | 0.0023 | - | - | - | - | 0.12 | 0.12 | 0.339 | 0.540 | Comparative Example |
| 20 | 0.067 | 0.23 | 2.63 | 0.010 | 0.0023 | 0.037 | 0.023 | 0.015 | 0.0021 | 0.0020 | 0.0025 | - | - | - | - | - | - | 0.505 | 0.313 | Comparative Example |
| 21 | 0.072 | 0.23 | 2.12 | 0.027 | 0.0013 | 0.029 | 0.030 | 0.008 | 0.0049 | 0.0020 | 0.0030 | - | 0.016 | - | - | - | - | 0.429 | 0.418 | Comparative Example |
| 22 | 0.074 | 0.14 | 2.14 | 0.006 | 0.0062 | 0.053 | 0.039 | 0.016 | 0.0036 | 0.0021 | 0.0022 | 0.0011 | - | - | - | 0.11 | - | 0.453 | 0.142 | Comparative Example |
| 23 | 0.051 | 0.26 | 2.13 | 0.007 | 0.0025 | 0.050 | 0.063 | 0.010 | 0.0034 | 0.0016 | 0.0026 | - | - | - | - | - | - | 0.406 | 0.189 | Comparative Example |
| 24 | 0.087 | 0.08 | 2.11 | 0.010 | 0.0032 | 0.041 | 0.032 | 0.033 | 0.0023 | 0.0024 | 0.0033 | - | - | - | - | - | - | 0.439 | 0.194 | Comparative Example |
| 25 | 0.075 | 0.18 | 2.07 | 0.007 | 0.0018 | 0.054 | 0.033 | 0.017 | 0.0076 | 0.0022 | 0.0036 | - | - | - | - | - | - | 0.420 | 0.232 | Comparative Example |
| 26 | 0.089 | 0.12 | 2.09 | 0.011 | 0.0020 | 0.034 | 0.015 | 0.016 | 0.0017 | 0.0028 | 0.0017 | 0.0047 | - | - | - | 0.16 | - | 0.469 | 0.750 | Comparative Example |
| 27 | 0.034 | 0.16 | 1.88 | 0.005 | 0.0027 | 0.049 | 0.033 | 0.014 | 0.0016 | 0.0009 | 0.0013 | - | - | - | - | - | 0.91 | 0.529 | 0.152 | Comparative Example |
| 28 | 0.087 | 0.22 | 1.91 | 0.004 | 0.0036 | 0.046 | 0.038 | 0.008 | 0.0029 | 0.0021 | 0.0026 | - | 0.220 | - | - | - | - | 0.449 | 0.205 | Comparative Example |
| 29 | 0.041 | 0.08 | 1.66 | 0.009 | 0.0017 | 0.026 | 0.042 | 0.008 | 0.0025 | 0.0012 | 0.0020 | - | - | - | - | 0.94 | - | 0.506 | 0.248 | Comparative Example |
| 30 | 0.088 | 0.25 | 2.08 | 0.005 | 0.0029 | 0.023 | 0.021 | 0.013 | 0.0031 | 0.0011 | 0.0038 | - | - | 0.34 | 0.24 | - | - | 0.473 | -0.035 | Comparative Example |
| 31 | 0.051 | 0.25 | 2.12 | 0.007 | 0.0012 | 0.021 | 0.017 | 0.014 | 0.0040 | 0.0028 | 0.0011 | - | - | 0.30 | 0.19 | - | 0.11 | 0.459 | 1.468 | Comparative Example |

| | | | | | | | | | | | | | | | | | | | | |
|---|---|---|---|---|---|---|---|---|---|---|---|---|---|---|---|---|---|---|---|---|
| *1: Ceq=C+Mn/6+(Cr+Mo+V)/5+(Cu+Ni)/15 *2: ACR=(Ca-(0.18+130×Ca)×O)/1.25/S In expressions *1 and *2, the element symbols represent the respective contents (mass%) of the elements. | | | | | | | | | | | | | | | | | | | | |

## Claims

1. A method of manufacturing a high-tensile strength steel comprising:
heating a steel slab having a component composition including C: 0.03 to 0.10 mass%, Si: 0.30 mass% or less, Mn: 1.60 to 2.30 mass%, P: 0.015 mass% or less, S: 0.005 mass% or less, Al: 0.005 to 0.06 mass%, Nb: 0.004 to 0.05 mass%, Ti: 0.005 to 0.02 mass%, N: 0.001 to 0.005 mass%, Ca: 0.0005 to 0.003 mass%, and optionally further comprising one or more selected from the group consisting of B: 0.0003 to 0.0025 mass%, V: 0.2 mass% or less, Cu: 1 mass% or less, Ni: 2 mass% or less, Cr: 0.7 mass% or less, and Mo: 0.7 mass% or less, and the balance of Fe and inevitable impurities so that Ca, S, and O satisfy the following expression (1): $0 < \left(Ca-\left(0.18+130⁢xCa\right)⁢xO\right) / 1.25 / S < 1$
wherein, Ca, S, and O represent the respective contents (mass%) of the elements, to 1050 to 1200°C;
hot-rolling the steel in such a manner that the cumulative rolling reduction in the temperature range of 950°C or higher is 30% or more and the cumulative rolling reduction in the temperature range of lower than 950°C is 30 to 70%; and then
cooling the steel from the hot-rolling finishing temperature to a cooling termination temperature of 600 to 450°C at a cooling rate of 5 to 45°C/sec and then cooling the steel from the first cooling termination temperature to a cooling termination temperature of 450°C or lower at a cooling rate of 1°C/sec or more and less than 5°C/sec.

2. The method of manufacturing a high-tensile strength steel according to Claim 1, wherein the steel after the second cooling is subjected to tempering at 450 to 650°C.

3. The method of manufacturing a high-tensile strength steel according to Claim 1 or 2, wherein the first cooling is performed at a cooling rate of 5 to 20°C/sec.

## Patentansprüche

1. Verfahren zur Herstellung eines Stahls mit hoher Reißfestigkeit, umfassend:
Erwärmen einer Stahlbramme, deren Bestandteil-Zusammensetzung Folgendes aufweist: 0,03 bis 0,10 Masseprozent C, 0,30 Masseprozent oder weniger Si, 1,60 bis 2,30 Masseprozent Mn, 0,015 Masseprozent oder weniger P, 0,005 Masseprozent oder weniger S, 0,005 bis 0,06 Masseprozent Al, 0,004 bis 0,05 Masseprozent Nb, 0,005 bis 0,02 Masseprozent Ti, 0,001 bis 0,005 Masseprozent N, 0,0005 bis 0,003 Masseprozent Ca, und gegebenenfalls zudem umfassend einen oder mehr Bestandteile, ausgewählt aus der Gruppe, bestehend aus 0,0003 bis 0,0025 Masseprozent B, 0,2 Masseprozent oder weniger V, 1 Masseprozent oder weniger Cu, 2 Masseprozent oder weniger Ni, 0,7 Masseprozent oder weniger Cr, und 0,7 Masseprozent oder weniger Mo, und als Rest Fe und unvermeidbare Verunreinigungen, so dass Ca, S, und O dem folgenden Ausdruck (1) entsprechen: $0 < \left(Ca-\left(0,18+130 x Ca\right) x O\right) / 1 , 25 / S < 1$
wobei Ca, S, und O den jeweiligen Inhalt (Masseprozent) der Elemente bei 1050 bis 1200°C umfasst;
Warmwalzen des Stahls auf eine Weise, dass die kumulative Walzreduktion im Temperaturenbereich von 950°C oder höher 30% oder mehr beträgt, und die kumulative Walzreduktion im Temperaturenbereich unter 950°C 30 bis 70% beträgt; und daraufhin Kühlen des Stahls von der Warmwalz-Endbearbeitungstemperatur zu einer Kühlbeendigungstemperatur von 600 bis 450°C bei einer Kühlgeschwindigkeit von 5 bis 45°C/sec und daraufhin Kühlen des Stahls von der ersten Kühlbeendigungstemperatur auf eine Kühlbeendigungstemperatur von 450° oder niedriger bei einer Kühlgeschwindigkeit von 1 °C/sec oder mehr und weniger als 5°C/sec.

2. Verfahren zur Herstellung eines Stahls mit hoher Reißfestigkeit nach Anspruch 1, wobei der Stahl nach dem eiten Kühlen bei 450 bis 650°C getempert wird.

3. Verfahren zur Herstellung eines Stahls mit hoher Reißfestigkeit nach Anspruch 1 oder 2, wobei das erste Kühlen bei einer Kühlgeschwindigkeit von 5 bis 20°C/sec erfolgt.

## Revendications

1. Procédé de fabrication d'un acier ayant une résistance à la traction élevée comprenant :
le chauffage d'une brame d'acier ayant une composition de composants incluant C : 0,03 à 0,10 % en masse, Si : 0,30 % en masse ou moins, Mn : 1,60 à 2,30 % en masse, P : 0,015 % en masse ou moins, S : 0,005 % en masse ou moins, Al : 0,005 à 0,06 % en masse, Nb : 0,004 à 0,05 % en masse, Ti : 0,005 à 0,02 % en masse, N : 0,001 à 0,005 % en masse, Ca : 0,0005 à 0,003 % en masse, et comprenant en outre éventuellement un ou plusieurs éléments choisis dans le groupe constitué de B : 0,0003 à 0,0025 % en masse, V : 0,2 % en masse ou moins, Cu : 1 % en masse ou moins, Ni : 2 % en masse ou moins, Cr : 0,7 % en masse ou moins et Mo : 0,7 % en masse ou moins, le reste étant du fer et d'inévitables impuretés de telle sorte que Ca, S et O satisfassent l'expression (1) suivante : $0 < \left(Ca-\left(0,18+130 x Ca\right) X O\right) / 1 , 25 / S < 1$
dans laquelle Ca, S et O représentent les teneurs respectives (% en masse) des éléments, à une température de 1050 à 1200°C ;
le laminage à chaud de l'acier de telle manière que la réduction cumulative du laminage dans la plage de températures de 950° ou plus est de 30 % ou plus et la réduction cumulative du laminage dans la plage de températures inférieure à 950° est de 30 à 70 % ; et, ensuite,
le refroidissement de l'acier de la température finale de laminage à chaud à une température de fin de refroidissement de 600 à 450°C à une vitesse de refroidissement de 5 à 45°C/s et ensuite, le refroidissement de l'acier de la première température de fin de refroidissement à une température de fin de refroidissement inférieure ou égale à 450°C à une vitesse de refroidissement de 1°C/s ou plus et inférieure à 5°C/s.

2. Procédé de fabrication d'un acier ayant une résistance à la traction élevée selon la revendication 1, dans lequel l'acier, après le second refroidissement, est soumis à un traitement de trempe à une température de 450 à 650°C.

3. Procédé de fabrication d'un acier ayant une résistance à la traction élevée selon la revendication 1 ou 2, dans lequel le premier refroidissement est effectué à une vitesse de refroidissement de 5 à 20°C/s.
